

# United States Patent

Frost et al.

[15] 3,668,100

[45] June 6, 1972

[54] **ELECTROPHORETIC COATING OF  
METAL SUBSTRATES USING  
ELEVATED PRESSURES**

[72] Inventors: **Lincoln J. Frost, La Salle; Arnd J. Stadler,**  
Park Forest, both of Ill.

[73] Assignee: **Continental Can Company, Inc., New**  
York, N.Y.

[22] Filed: **July 1, 1970**

[21] Appl. No.: **51,692**

[52] U.S. Cl. .... **204/181**

[51] Int. Cl. .... **B01k 5/02, C23b 13/00**

[58] Field of Search ..... **204/181**

[56]

## References Cited

### UNITED STATES PATENTS

3,476,666 11/1969 Bell et al..... 204/181  
3,496,082 2/1970 Orem et al..... 204/181

*Primary Examiner*—Howard S. Williams

*Attorney*—Paul Shapiro, Joseph E. Kerwin and William A. Dittmann

[57]

## ABSTRACT

In a process of electrophoretic coating of electrically conductive surfaces with organic resins, the amount of resin deposited is substantially increased by conducting the electrophoretic deposition at pressures above atmospheric.

5 Claims, No Drawings

## ELECTROPHORETIC COATING OF METAL SUBSTRATES USING ELEVATED PRESSURES

### BACKGROUND OF THE INVENTION

#### 1. Field of the Invention

This invention relates to coating the electrically conductive surface areas of articles, and in particular, to coating metal articles by electrophoretic deposition of organic film-forming material.

#### 2. The Prior Art

In the manufacture of cans, the blank stock is ordinarily coated while the material is flat. Since the cans are welded after this operation, the edges of the blank stock are cleaned so that the welding process forms an impervious joint. After welding, it is necessary to apply side striping or coating to the exposed cut edges of the metal portions that form the can side-seam to prevent corrosion and/or product contamination on the interior portion of the can and for esthetic appeal on the exterior portion of the can body.

One method that has been proposed for coating these exposed bare metal surface areas of the can side-seam is electrophoretic deposition. In this coating method, the metal surface to be coated is immersed in an electrophoretic bath which generally consists of particles of an organic-film forming polymeric coating materials which are suspended in an aqueous electrolytic solution. The exposed bare conducting surface areas of the surface to be coated serve as one electrode of the electrocoating bath. When a potential of the required polarity is applied between the exposed surface areas of the article to be coated and a second electrode which completes the electrical circuit and is dipped into the aqueous coating suspension, the particles of the coating material are deposited on the metal surface's exposed areas in the form of a uniform layer.

Electrophoretic deposition has not been practiced to date for coating the bare cut edges of can side-seams due to the fact that the coating thicknesses required i.e. about 6 to 8 mils cannot be achieved using conventional electrophoretic deposition processes. Using such conventional electrophoretic coating techniques the maximum coating thickness that can be achieved are in the range of 2 to 4 mils.

### SUMMARY OF THE INVENTION

In accordance with the present invention, there is provided a method for the electrophoretic coating of metal surfaces which includes contacting the surface to be coated with an electrophoretic bath having a synthetic polymer resin dispersed therein and electrophoretically depositing the synthetic polymer resin on the exposed electrically conductive areas of the surface at a pressure greater than atmospheric.

As will hereinafter be illustrated, the step of electrophoretically depositing the synthetic polymer resin at pressures greater than atmospheric results in a deposited coating of substantially greater thickness when compared to similar coated surfaces which have not been subjected to elevated pressures.

### PREFERRED EMBODIMENTS

To effect the electrophoretic coating of metal surfaces in accordance with the present invention, a synthetic polymer resin containing electrolyte is contacted with the metal surface to be coated. To effect deposition of the polymeric coating material from the electrophoretic coating bath, an electrical current is caused to flow between the metal surface to be coated and a suitable electrode immersed in the electrophoretic coating bath by establishing a DC potential between the metal surface and the electrode and permitting the electrical current to flow until the electrically conducting surface areas of the metal have been coated with polymer deposited from the bath. In the case of can bodies which have been enamel coated prior to exposure to the bath, the electrophoretic polymer coating is deposited only on those areas of the enamel coated bodies where bare metal is exposed such as the cut edges of the metal portions that form the side seam

of the can. Due to the electrical insulating properties of the enamel coating, no polymer is electrodeposited on the enamel coated areas of the can body.

During the electrodeposition process in order to achieve coating deposits of substantially increased thickness in accordance with the process of the present invention, the pressure of the atmosphere surrounding the article surface immersed in the electrophoretic bath is raised above atmospheric pressure. Generally the pressure required to achieve the improved results is maintained in the range of about 1 to about 50 pounds per square inch (psi), pressures in the range of 2 to 20 psi being preferred.

The electrical potential applied in the electrophoretic bath to deposit the repair coating is controlled below the value at which dielectric breakdown of the deposited coating occurs and may range from between about 20 volts to about 2,000 volts per inch of electrode spacing.

The time required to effect repair coating is not critical since coating of the exposed portions of the metal surface to be coated begins in a fraction of a second from the point where the electrical circuit is closed and stops when the insulating polymeric coating is deposited. Thus, the time used to effect the deposition of the coating may range between about 1 second and about 100 seconds and preferably about 2 to 20 seconds.

The current density selected for the electrophoretic deposition varies and generally will depend upon such parameters as the selected voltage, the conductivity of the electrophoretic coating bath, and the time allotted for the formation of a coating. Generally, the electrophoretic processing voltage is varied from about 100 to about 900 volts per inch of electrode spacing to coat exposed metal areas within a reasonable time, e.g., about 2 to about 5 seconds.

The temperature of the electrophoretic bath is not critical other than the boiling and freezing point of the colloidal suspension used as the electrophoretic bath. For practical applications it is preferred to use temperatures in the range of about 15° to about 60° C.

The electrophoretic coating bath used in the process of the present invention is a colloidal suspension consisting of charged particles of a synthetic polymer resin dispersed in a suitable liquid electrolyte. Preferably, the resins utilized in the electrophoretic coating baths of the present invention are any resins, thermoplastic or thermosetting, which have free carboxylic acid groups or hydroxyl groups.

Illustrative examples of resins which have free carboxylic acid or hydroxyl groups which may be used in the electrophoretic baths include acrylic resins such as polyacrylic acid, polymers of hydroxyalkyl esters of  $\alpha,\beta$ -ethylenically unsaturated carboxylic acids, such as poly (2-hydroxyethyl acrylate), poly (2-hydroxypropyl methacrylate), copolymers of ethylene and  $\alpha,\beta$ -ethylenically unsaturated carboxylic acids, such as ethylene/acrylic acid copolymers, ethylene/methacrylic acid copolymers, polymers of mono- and di-esters of unsaturated dicarboxylic acids, such as maleic acid, fumaric acid, and itaconic acid, in which at least one of the esterifying groups contains a hydroxyl group, such as polymers of mono (2-hydroxyethyl) maleate, mono (2-hydroxypropyl) fumarate, and the like.

The above described resins may be further blended with an alkoxy methyl aminoplast, such as a methoxy melamine ester, methoxy methyl benzoguanamine ether, or butylated urea/formaldehyde resin to obtain heat hardenable resin formulations containing about 60 to 95 percent of the carboxylic acid or hydroxyl group containing resin and about 5 to about 40 percent by weight of the aminoplast resin.

A stable dispersion of these resins in water is made in the presence of ammonia or triethanolamine. An anionic surface active agent may be utilized if necessary.

The concentration of resin solids in the electrophoretic bath may be widely varied. In general, the solids content of the synthetic polymer resin in the bath may be varied from 2 to 15 percent by weight.

After the synthetic polymer resin is electrophoretically deposited on the metal surface, the article is separated from the bath and rinsed with water to remove adhering portions of the coating solution. Following rinsing, the electrophoretically coated article is placed in an oven and baked at an elevated temperature, e.g., about 300° to about 450° F for about 1 to about 20 minutes to remove all volatile material and cure the electrophoretically deposited coating to a hardened film.

To illustrate the manner in which the present invention may be carried out, the following examples are given. It is to be understood, however, that the examples are for the purpose of illustration, and the invention is not to be regarded as limited to any of the specific materials or conditions recited therein.

#### EXAMPLE I

Blanks were cut from an epoxy-urea/formaldehyde resin coated metal sheet and fabricated into open cylinders having a welded side seam to form the body of a container wherein the enamel coated side of the blanks formed the interior of the container. The cut edge of the metal portions that formed the seam was bare metal. The container body was closed at one end with end closures formed from a similarly enamel coated sheet which was double seamed to the cylinder wall.

The container was then filled with electrophoretic bath consisting of 5 percent resin solids dispersed in an aqueous triethanolamine solution. The resin solids were composed of a mixture of 80 percent by weight of a 70% hydroxyl functional acrylic resin having a molecular weight of about 30,000 and 20 percent by weight of a melamine/formaldehyde resin.

A steel electrode was placed in the container in a position so that all the points on the electrode surface were  $\frac{1}{4}$  inch to  $1\frac{1}{2}$  inches from the nearest point on the inside of the container. The container was then placed in a pressure vessel and the vessel closed.

A current having a potential of about 465 volts was applied across the electrode in the container for about 4 seconds, the container being the anode. The temperature of the bath was about 110° F after the application of the current, the container was inverted to remove the bath liquid. The inverted container was rinsed with water and baked for 2 minutes at 250° F and 4 minutes at 385° F in a forced air oven.

A series of similarly fabricated containers were coated following the above procedure using pressures varying from 2 to 20 psi.

For purposes of comparison, the above coating procedure was also conducted at atmospheric pressure (0 psi). The coating weights deposited are recorded in table I below. A coating weight of about 70 milligrams is approximately equivalent to a deposited coating thickness of 8 mils.

TABLE I

| Test No.                   | 1  | 2  | 3  | 4  | Control |
|----------------------------|----|----|----|----|---------|
| Pressure (psi)             | 2  | 5  | 10 | 20 | 0       |
| Coating Weight Gain (mgs.) | 45 | 48 | 57 | 70 | 37      |

By reference to table I it is immediately apparent the cans electrophoretically coated at elevated pressures in accordance with the present invention show a substantially greater gain in coating weight when compared to similar cans coated under ambient or atmospheric pressures.

#### EXAMPLE II

The procedure of example I was repeated with the exception that the acrylic resin used in the electrophoretic bath had a molecular weight of about 15,000. In this test series the effect of subatmospheric pressure on deposition rate was also studied. The results of this series of tests is recorded in table II below. Control tests (0 psi) and subatmospheric pressure tests are designated by the symbol "C."

TABLE II

| Test No.                   | 5   | 6   | 7   | C <sub>1</sub> | C <sub>2</sub> | C <sub>3</sub> | C <sub>4</sub> |
|----------------------------|-----|-----|-----|----------------|----------------|----------------|----------------|
| Pressure (psi)             | 10  | 20  | 20  | 0              | 0              | 20*            | 10*            |
| Coating Weight Gain (mgs.) | 111 | 127 | 140 | 54             | 81             | 26             | 51             |

\* Subatmospheric pressure

#### EXAMPLE III

The procedure of example I was repeated with the exception that Shell DX-31, the reaction product of an epoxy resin, bisphenol A, benzoic acid and a linseed oil fatty acid was used as the resin vehicle in the electrophoretic bath at a solids content of 9.8 percent. The results of this series of tests is recorded in table III below.

TABLE III

| Test No.                   | 8  | 9  | 10 | 11 | C <sub>5</sub> |
|----------------------------|----|----|----|----|----------------|
| Pressure (psi)             | 5  | 10 | 20 | 50 | 0              |
| Coating Weight Gain (mgs.) | 62 | 66 | 76 | 98 | 54             |

What is claimed is:

1. A method of electrophoretically coating articles having electrically conductive surfaces which comprises the steps of:
  - a. causing the electrically conductive surface of the article to be coated to be immersed in an electrophoretic bath having charged particles of an organic coating material dispersed therein, the electrically conductive article surface serving as a first electrode;
  - b. raising the pressure of the atmosphere above the bath to a pressure greater than atmospheric pressure and then;
  - c. causing a second electrode to contact said electrophoretic bath and causing a direct electric current to flow in the bath between the electrically conductive article surface and the second electrode until the electrically conducting surface areas of the article have been electrophoretically coated with the organic coating material.
2. The method of claim 1 wherein the pressure in the atmosphere above the bath is raised between about 1 to about 100 psi during the electrophoretic coating of the article.
3. The method of claim 1 wherein the organic coating material is a thermoplastic resin.
4. The method of claim 1 wherein the organic coating material is a thermosetting resin.
5. The method of claim 4 wherein the thermosetting resin electrophoretically coated surface is heated to harden the electrophoretically deposited coating.

\* \* \* \* \*